

# United States Patent [19]

[ 19 ]

Elliott et al.

[11] 3,844,963

[45] Oct. 29, 1974

[54] LUBRICANTS

[75] Inventors: **John Scotchford Elliott; Gerald John Joseph Jayne; Patrick Robert James Foliard**, all of London, England

[73] Assignee: **Edwin Cooper & Company Limited,**  
London, England

[22] Filed: July 5, 1972

[21] Appl. No.: 269,205

### [30] Foreign Application Priority Data

July 6, 1971 Great Britain ..... 31634/71

[52] U.S. Cl. .... 252/46.7, 252/400 A

[51] Int. Cl. .... C10m 1/48

[58] **Field of Search**..... 252/46.7, 400 A

[ 56 ] References Cited

UNITED STATES PATENTS

|           |         |                       |          |
|-----------|---------|-----------------------|----------|
| 2,648,696 | 8/1953  | Whetstone .....       | 260/935  |
| 2,743,235 | 4/1956  | McDermott .....       | 252/46.7 |
| 3,317,425 | 5/1967  | Hasserodt et al. .... | 252/46.7 |
| 3,446,738 | 5/1969  | Chao et al. ....      | 252/46.7 |
| 3,537,998 | 11/1970 | Lowe .....            | 252/46.7 |

*Primary Examiner*—Helen M. S. Snead  
*Attorney, Agent, or Firm*—Bacon & Thomas

[57]

## ABSTRACT

A lubricant composition comprises a major amount of lubricating oil and a minor amount of one or more oil-soluble dithiophosphoric acid derivatives having the general formula:



wherein  $R^3$  is a mono- or di-*valent* aliphatic or aromatic group;  $X$  is an oxygen or sulphur atom;  $R^4$  is an alkyl group;  $R^1$  and  $R^2$  are the same or different and are alkyl, alkaryl, aryl or aralkyl groups or alkenyl and  $n$  is 0 when  $R^3$  is a monovalent group or is 1 when  $R^3$  is a divalent group.

The dithiophosphoric acid derivatives, certain of which are novel compounds, function as antioxidants, load carrying and antiwear additives in the lubricant compositions.

## 8 Claims, No Drawings

1  
LUBRICANTS

This invention relates to lubricants and in particular to lubricants containing S-carbamoyl dithiophosphates.

Many dithiophosphate compounds have been employed as additives in lubricants to reduce wear and to act as antioxidants, the most widely used additives being the zinc salts of 0,0'-dihydrocarbyl dithiophosphoric acids. These zinc salts have been widely used for many years and have proved to be very useful in formulating lubricants. Nevertheless, the zinc salts suffer from a number of disadvantages and in particular cannot be employed in ash-free lubricants since the zinc content is a source of ash. Consequently efforts have been made to prepare ash-free dithiophosphoric acid derivatives which can be employed as antioxidants, load carrying and antiwear additives.

In U.S. Pat. No. 3,537,998 there are described certain dithiophosphoric acid derivatives useful as antioxidant, antiwear and extreme pressure additives, which derivatives have the formula:



wherein Ar is arylene of from 6 to 12 carbon atoms and R is a hydrocarbyl group, substantially free of aliphatic unsaturation, having from 12 to 30 carbon atoms.

It is desirable that dithiophosphate lubricant additives in addition to possessing antioxidant, load-carrying and antiwear properties, should not be unduly prone to form deposits in oil solution at the elevated temperatures at which internal combustion engines are normally operated, e.g., up to 130°C.

The present invention provides lubricants containing ash-free dithiophosphoric acid derivatives, some of which are novel compounds, having a reduced tendency to form deposits composed of oil-insoluble diisothiocyanate decomposition products.

Accordingly the present invention provides a lubricant composition comprising a major amount of lubricating oil and a minor amount of one or more oil-soluble dithiophosphoric acid derivatives having the general formula:



wherein R<sup>3</sup> is a mono- or di-va lent aliphatic or aromatic group; X is an oxygen or sulphur atom; R<sup>4</sup> is an alkyl group; R<sup>1</sup> and R<sup>2</sup> are the same or different and are alkyl, alkaryl, aryl or aralkyl groups or alkenyl and n is 0 when R<sup>3</sup> is a monovalent group or is 1 when R<sup>3</sup> is a divalent group.

The additives of the present invention may contain as a contaminant, a small proportion of isothiocyanate decomposition products.

The groups R<sup>1</sup> and R<sup>2</sup> are preferably alkyl, alkaryl or aralkyl groups, and may contain from 1 to 30, preferably 4 to 18, carbon atoms. The group R<sup>4</sup> may contain from 1 to 30, preferably 2 to 22, more preferably 4 to 13, carbon atoms. The group R<sup>3</sup> is preferably a monovalent alkyl group containing from 1 to 18 carbon

## 2

atoms or a di-va lent aryl group, optionally bearing one or more alkyl substituents, which contains from 6 to 24 carbon atoms.

It will be understood that the carbon atom content of the groups R<sup>1</sup>, R<sup>2</sup>, R<sup>3</sup> and R<sup>4</sup> will be selected so as to provide an oil-soluble compound.

The dithiophosphoric acid derivatives employed in the lubricants of the present invention may be prepared by reacting an isocyanate compound, as more fully described hereinafter, with a dithiophosphoric acid. The dithiophosphoric acid starting materials may be prepared by reaction of 1 mole of phosphorus pentasulfide with 4 moles of an alcohol or mixture of alcohols, a phenol or mixture of phenols or a mixture of one or more alcohols and one or more phenols in accordance with techniques well-known in the preparation of the zinc salts of 0,0'-dihydrocarbyl dithiophosphoric acids hereinbefore described. Thus, the nature of the alcohol and/or phenol employed will determine the nature of the groups R<sup>1</sup> and R<sup>2</sup> in the additives of the present invention. Examples of alcohols which may be used include:

ethanol  
n-propanol  
isopropanol  
n-butanol  
isobutanol  
amyl alcohol, including mixed amyl alcohols  
mixtures of alcohols, derived from the "OXO" process

decanol  
dodecanol  
lauryl alcohol  
Suitable phenols include:

p-tert-butyl phenol  
heptyl phenol  
p-nonyl phenol  
m-pentadecyl phenol  
polyalkylene substituted phenols preferably derived from polypropylene, especially propylene tetramer, and polyisobutylenes having molecular weights up to 2,500.

Examples of suitable mixtures of alcohols and phenols include:

mixtures of isobutanol with mixed amyl alcohols  
isopropyl alcohol and 1-methyl heptanol  
isopropyl alcohol and 2-ethyl hexanol  
isobutanol and 2-ethyl hexanol  
amyl alcohol and p-tertiary octyl phenol

The dithiophosphoric acids prepared in the above described manner are reacted with the isocyanate compound.

The isocyanate compound which may be employed in the preparation of the additives can be a mono-isocyanate, preferably an aliphatic mono-isocyanate, of the formula:



Suitable mono-isocyanates which may be used to prepare S-carbamoyl dithiophosphates which may be used in the present invention include:

methyl isocyanate  
ethyl isocyanate  
n-propyl isocyanate  
isopropyl isocyanate  
n-butyl isocyanate  
tert-butyl isocyanate

octadecyl isocyanate  
allyl isocyanate  
phenyl isocyanate

Alternatively, the isocyanate compound can have the formula:



wherein  $R^3$ ,  $R^4$  and  $X$  are as hereinbefore defined. Isocyanates of the latter formula may be prepared by reacting one of the isocyanate groups of a di-isocyanate with an alcohol or mercaptan.

In a further alternative preparation of the additives used in the present invention a dithiophosphoric acid is reacted with one of the isocyanate groups of a di-isocyanate and the remaining isocyanate group is reacted with an alcohol or mercaptan.

Suitable di-isocyanates include toluene 2,4, di-isocyanate, which is particularly preferred.

Other di-isocyanates are:

diphenyl methane di-isocyanate  
3-3'-dimethyl-4,4' biphenylene di-isocyanate  
trimethyl hexamethylene di-isocyanate  
hexa methylene di-isocyanate

Compounds which may be reacted with the di-isocyanate include:

methanol  
ethanol  
isopropanol  
n-butanol  
isobutanol  
amyl alcohol  
n-hexyl alcohol  
2-ethylhexanol  
3,5,5-trimethyl-hexanol  
isodecanol  
n-decanol  
dodecanol  
isotridecanol

mixed straight chain alcohols sold under the trade name "Alfol" containing up to 22 carbon atoms, and n-dodecyl mercaptan.

The temperature at which the additives of the present invention are prepared may be varied according to the preparative route chosen. In order to obtain the optimum antioxidant performance, load-carrying ability and to minimise deposit formation at elevated temperatures it is preferred to carry out the reaction with the dithiophosphoric acid at about 75° - 80°C., although temperatures of up to 100°C. or as low as ambient temperature may be employed, if desired.

Each of the reactions carried out in the preparation of the additives is conveniently carried out at atmospheric pressure. However, any or all of the reactions may be carried out, if desired, at pressures above or below atmospheric.

The lubricants of the present invention may contain from 0.1 to 10%, preferably from 0.5 to 5%, by weight of the dithiophosphoric acid derivatives. The lubricants may also contain other additives of the type conventionally used in lubricants, especially ash-free additives. Such additives include antioxidants and antiwear additives (additional to the dithiophosphoric acid derivatives) and corrosion inhibitors, detergents, dispersants, viscosity index improvers, extreme pressure additives or any combination thereof.

Suitable additional antioxidants are phenothiazine, optionally substituted on one or both benzene nuclei and/or the nitrogen atom, a hindered phenol or a hindered bis-phenol or a secondary amine having two aromatic nuclei attached to the nitrogen atom. In one aspect of the invention the additional antioxidant is a secondary amine having two aromatic nuclei attached to the nitrogen atom, in which one or both of the aromatic nuclei bear one or more alkyl groups, particularly alkyl groups containing from 4 to 12, more preferably 8 or 9, carbon atoms. Examples of such amines are mono-octyl phenyl- $\alpha$ -naphthylamines and mono-octyl phenyl- $\beta$ -naphthylamines, particularly N-p-t-octyl phenyl- $\alpha$ -naphthylamine and N-p-t-octyl phenyl- $\beta$ -naphthylamine; and mono-nonyl phenyl- $\alpha$ -naphthylamines and mono-nonyl phenyl- $\beta$ -naphthylamines. Other amines are diphenylamine and mono- or di-alkyl diphenylamines, particular examples being di-octyl and di-nonyl diphenylamines, especially the p-p' isomers. These secondary amines may be used in an amount of from 0.1% by weight, preferably 0.2% to 5% by weight. Other ash-free antioxidants which may be used include the trithiopyrophosphate additives described in British Pat. No. 1,254,554, and in German

Offenlegungsschrift No. 2,162,180 and copending United States application Ser. No. 252,254 filed May 11, 1972.

Suitable corrosion inhibitors include benzotriazole or a derivative thereof, an aliphatic carboxylic acid, a dicarboxylic acid, for example, dodecanyl succinic acid, mercaptobenzothiazole and benzothiazole disulphide.

Suitable detergents include an alkaline earth metal petroleum or alkyl benzene sulphonate, carboxylate, salicylate or naphthenate, any of which may be overbased with an alkaline earth metal carbonate. Other suitable detergents, which may also be overbased, include a phosphosulphurised hydrocarbon and an alkyl phenol which has been neutralised by an alkaline earth metal base.

A suitable dispersant is a long chain hydrocarbon substituted by a polyamine group attached thereto either directly or through an amide or imide link, as described in British Pat. Nos. 1,068,235 and 1,121,641.

A typical viscosity index improver which may be used in this invention is a copolymer of a mixture of monomers, which monomers are esters of acrylic or methacrylic acid. Other unsaturated monomers such as N-vinyl pyrrolidone, diethylamino-ethyl methacrylate or fumaric acid may be included in the mixture to give viscosity index improvers having dispersant properties.

In certain cases, e.g., for ease of transport, it may be desirable to prepare more concentrated solutions of the dithiophosphoric acid derivatives which can be diluted with additional lubricating oil before being used. These more concentrated solutions may be oil concentrates or additive packages, i.e., may be, respectively concentrated solutions of one or more dithiophosphoric acid derivatives or concentrated solutions of mixtures of one or more dithiophosphoric acid derivatives and one or more known additives. Accordingly, in a further embodiment of the invention there is provided an oil concentrate or additive package comprising from 10% to 70%, more preferably 20% to 50%, by weight of a lubricating oil having dissolved therein from 90% to 30%, more preferably 80% to 50%, by weight of one or more

of the dithiophosphoric acid derivatives, optionally together with one or more known additives.

The lubricating oil employed in the lubricants, oil concentrates and additive packages of the present invention may be a mineral oil of lubricating viscosity of well-known type. Alternatively, a synthetic ester-based oil may be used as the lubricating oil. Suitable synthetic ester oils are described in British Pat. Nos. 930,136 and 1,205,177.

As hereinbefore stated certain of the dithiophosphoric acid derivatives employed in the lubricants are novel compounds. The present invention therefore includes in another aspect novel dithiophosphoric acid derivatives suitable for use as lubricant additives, having the general formula:



wherein  $R^1$ ,  $R^2$ ,  $R^3$  as a di-va lent group,  $R^4$  and  $X$  are as hereinbefore defined.

In yet another aspect of the present invention there is provided a process for the preparation of a dithiophosphoric acid derivative, which process comprises reacting an isocyanate compound of the formula:



with a compound of formula:



to produce a dithiophosphoric acid derivative having the general formula:



wherein  $R^1$ ,  $R^2$ ,  $R^3$  as a di-va lent group,  $R^4$  and  $X$  are as hereinbefore defined.

Moreover the present invention further provides a process for the preparation of a dithiophosphoric acid derivative, which process comprises reacting a compound of the formula:



with one of the isocyanate groups of a di-isocyanate and thereafter reacting the remaining isocyanate group with an alcohol or mercaptan.

It is to be understood that the invention also includes a dithiophosphoric acid derivatives when produced by either of the above processes.

The preparation of dithiophosphoric acid derivatives which may be used in lubricants in accordance with the

present invention will now be illustrated with reference to the following non-limiting examples.

#### EXAMPLE 1

5 Ethyl isocyanate (13.8g. 0.2m) was added dropwise to stirred di-tridecyl dithiophosphoric acid (110g. 0.2m) over a period of about 1 hour, the temperature of the reaction mixture being maintained at 70°-85°C. After each addition an exotherm was noticed.

10 When the addition was complete the product was allowed to cool slowly, with stirring, to yield 120g. (97%) of a light green mobile liquid.

|    |                          |           |            |           |
|----|--------------------------|-----------|------------|-----------|
| 15 | Analysis:                | 5.47 % P. | 11.16 % S. | 2.16 % N. |
|    | Theory                   | 5.49 % P. | 11.32 % S. | 2.48 % N. |
|    | Timken O.K. load 45 lbs. |           |            |           |

#### EXAMPLE 2

a. Isobutanol (74g. 1.0m) was added slowly, with stirring, to toluene di-isocyanate (174g. 1.0m) maintained at 70°-80°C. A strongly exothermic reaction followed each addition. Heating was then continued for 1 hour at 70°-80°C. followed by 1/2 hour at 110°C.

25 b. The reaction product of (a) above (70g) was added to di-nonylphenyl dithiophosphoric acid (145.8g.) in a glass flask over 1 hour while increasing the temperature to 80°-90°C. Thereafter the reaction was continued for a further 1 hour to yield 212g (98%) of a dark yellow liquid.

|    |                          |           |           |           |
|----|--------------------------|-----------|-----------|-----------|
| 30 | Analysis                 | 3.63 % N. | 3.98 % P. | 8.1 % S.  |
|    | Theory                   | 3.58 % N. | 3.97 % P. | 8.18 % S. |
|    | Timken O.K. load 60 lbs. |           |           |           |

#### EXAMPLE 3

Di-isobutyl dithiophosphoric acid (250g. 1m) was added to toluene di-isocyanate (174g. 1m) from a tap funnel over a period of 3/4 hour at 70°-80°C. After being left for 2 hours, with stirring, 2-ethylhexanol (143g. 1.1m) was added dropwise over a period of 1 hour. After a further 1/2 hour, stirring and heating was stopped, the product was filtered and stripped to 120°C. and 4 torr to yield 525 g. (96.3%).

|    |                          |           |           |            |
|----|--------------------------|-----------|-----------|------------|
| 55 | Analysis:                | 5.67 % P. | 4.95 % N. | 11.12 % S. |
|    | Theory                   | 5.67 % P. | 5.14 % N. | 11.72 % S. |
|    | Timken O.K. load 45 lbs. |           |           |            |

#### EXAMPLE 4

60 Isobutanol (14.8g., 0.2m) was added dropwise over 3/4 hour to toluene di-isocyanate (34.8g., 0.2m.), initially at 70°-80°C., causing the temperature to rise briefly to 110°C. 0.0'-di-tridecyl dithiophosphoric acid (110.2g., 0.2m) was then added, dropwise over one hour, with the temperature being maintained at 70°-80°C. A further quantity of isobutanol (1.5g., 10%) was then added to ensure that there was no free isocyanate in the product, and the mixture stirred for

one hour to yield 157g. (97.5%) of a greenish yellow liquid containing 3.97%P (theory 4.18%).

Timken O.K. load = 50 lbs.

#### EXAMPLE 5

a. Toluene di-isocyanate (174g., 1.0m) was heated to approximately 105°C. and 0,0'-di-isobutyl dithiophosphoric acid (250g., 1.0m) run in over 1/4 hour and left to react for a further 2 1/4 hours at 105°C.

b. To 100g. (0.24m.) of the product of (a) was added n-dodecyl mercaptan (47.5g., 0.24m) over 20 minutes at approximately 105°C. After stirring for a further 1/2 hour the product was cooled to yield 146g. (99%) of an olive green liquid containing 5.0%P and 16.4%S (theory 5.02% and 15.55% respectively).

#### EXAMPLE 6

3,5,5-Trimethyl hexanol (57.6g., 0.4m) was added to toluene di-isocyanate (69.6g., 0.4m.) at a temperature of 70°-80°C. and 0,0'-di-isobutyl dithiophosphoric acid (106g., 0.4m.) was added to the reaction product dropwise over a one hour period, followed by reaction for a further 1 1/4 hours. A yield of 223g. (95.5%) of a dark grey/green semi-solid containing 5.85%P (theory 5.52%) was obtained.

Timken O.K. load = 27 lbs.

#### EXAMPLE 7

Toluene di-isocyanate (69.6g., 0.4m.) was added to tridecanol (80.0g., 0.4m.) at 70°-80°C., and to the reaction product was added 0,0'-di-isobutyl dithiophosphoric acid (106.8g., 0.4m.) dropwise over 3/4 hour. The reaction was continued with stirring for a further hour to yield 245g. (99%) of a green, slightly viscous liquid containing 5.44%P (theory 5.04%).

Timken O.K. load = 30 lbs.

#### EXAMPLE 8

Tridecanol (40.0g., 0.2m.) was added to toluene di-isocyanate (34.8g., 0.2m.) over 1/2 hour at a temperature of 70°-80°C. and the product stirred for a further 1/2 hour. To the product was then added 0,0'-di-isobutyl dithiophosphoric acid (55.6g., 0.2m.) over 3/4 hour followed by a further 4.0g. (10%) of tridecanol and the reaction continued for a further one hour to yield 119g. (95%) of an olive green liquid containing 5.00%P (theory 5.04%).

Timken O.K. load = 45 lbs.

#### EXAMPLE 9

An 0,0'-dialkyl dithiophosphoric acid was prepared by reaction of  $P_2S_5$  with Alfol 20-22 (a commercially available mixture of alcohols containing 20-22 carbon atoms). To toluene di-isocyanate (34.8g., 0.2m.) was added, in bulk, 2-ethylhexanol (26g., 0.2m.), causing an exotherm. To the product was added the 0,0'-di-Alfol 20-22 dithiophosphoric acid (150g., 0.2m.), after melting, causing the temperature to rise to 50°C. The total addition time of the dithiophosphoric acid was 3/4 hour, after which the reaction was continued for a further 1 1/2 hours to yield 205g. (97.5%) of a grey/green solid containing 2.77%P (theory 2.93%).

Timken O.K. load = 60 lbs.

#### EXAMPLE 10

a. Isobutanol (74.0g., 1.0m.) was added dropwise to toluene di-isocyanate (174g., 1.0m.) over 3/4 hour, dur-

ing which time the initial temperature of 30°C. rose to 80°C. due to the strong exotherm. The reaction was continued, with stirring, for a further one hour.

b. To the reaction product of (a) (71.0g., 0.5m.) was added 0,0'-di-tridecyl dithiophosphoric acid (276g., 0.5m.) over 3/4 hour, an exotherm being noticed. The reaction temperature was 35°C. The final product was a light green liquid containing 4.72%P and 9.7%S (theory 4.18% and 8.62% respectively) and was obtained in a yield of 333g. (96%).

Timken O.K. load = 45 lbs.

#### EXAMPLE 11

To the reaction product (71.0g., 0.5m.) of Example 15 10(a) was added 0,0'-di-nonylphenyl dithiophosphoric acid (260g., 0.5m.) at 30°C. over 3/4 hour. The reaction was continued for a further one hour at 35°C. to yield 320g. (96.5%) of a yellow viscous liquid containing 4.44%P and 9.6%S (theory 3.96% and 8.18% respectively).

Timken O.K. load = 60 lbs.

#### EXAMPLE 12

a. Isobutanol (74g., 1.0m.) was added slowly, with stirring, to toluene di-isocyanate (174g., 1.0m.) maintained at 70°-80°C. over a period of 1 hour. Thereafter, reaction was continued for a further 1 hour.

b. To 70g. (0.282m.) of the reaction product of (a) above was added, 0,0'-di-tridecyl dithiophosphoric acid (145.8g., 0.282m.) over one hour, with the reaction temperature at 70°-80°C. The product was finally stirred at the same temperature for a further one hour to yield 213.3g. (98.5%) of a yellow/green liquid containing 4.22%P and 8.62%S (theory 4.18% and 8.53% respectively).

Timken O.K. load = 45 lbs.

#### EXAMPLE 13

Isobutanol (14.8g., 0.2m.) was added in bulk to toluene di-isocyanate (69.6g., 0.4m.) and reacted for one hour at 30°-45°C. 0,0'-di-2-ethylhexyl dithiophosphoric acid (76.8g., 0.2m.) was added dropwise over 3/4 hour at 30°C. and reaction continued for 1/2 hour. To 129g. of the resulting product was added, at 25°C., mole equivalents of isobutanol (12.3g.) and 0,0'-di-2-ethylhexyl dithiophosphoric acid (63.6g.) over a period of 3/4 hour. After reacting for 1 1/2 hours at 25°C. there was obtained 201g. of a mobile, light green liquid containing 4.75%P (theory 5.15%).

#### EXAMPLE 14

Toluene di-isocyanate (69.6g., 0.4m.) and 2-ethylhexanol (26.0g., 0.2m.) were reacted for 1 hour at about 30°-45°C. 0,0'-di-2-ethylhexyl dithiophosphoric acid (76.8g., 0.2m.) was then added dropwise over 3/4 hour at 30°C. and reaction continued for 1 hour. To 156g. of the resulting product were added mole equivalents of 0,0'-di-2-ethylhexyl dithiophosphoric acid (67.9g.) and 2-ethylhexanol (22.4g.) and reaction continued, with stirring, for 2 hours at a temperature of 20°C. There was obtained 235g., (95.4%) of a green liquid containing 4.15%P (theory 4.71%).

Timken O.K. load = 35 lbs.

#### EXAMPLE 15

Toluene di-isocyanate (69.6g., 0.4m.) and isobutanol (29.6g., 0.4m.) were reacted for 2 hours, the tempera-

ture exotherming to 75°C. at one stage. There was then added, at 30°C. over  $\frac{1}{4}$  hour, 132.8g. (0.4m.) of an 0,0'-dialkyl dithiophosphoric acid prepared from  $P_2S_5$  and Alfol 6 (commercially available mixture of alcohols having about 6 carbon atoms). Reaction was continued, with stirring, for a further one hour to yield 215g. (92.6%) of an olive green liquid containing 5.93%P (theory 5.68%).

#### EXAMPLE 16

Toluene di-isocyanate (69.6g., 0.4m.) and tridecanol (80.0g., 0.4m.) were reacted together and 0,0'-di-Alfol 6 dithiophosphoric acid (132.6g., 0.4m.) added over  $\frac{1}{4}$  hour, with the temperature at 30°-35°C. The reaction was continued for a further 1 hour to yield 270g. (96%) of a light green liquid containing 4.49%P (theory 4.61%).

Timken O.K. load = 50 lbs.

#### EXAMPLE 17

The procedure of Example 16 was repeated using toluene di-isocyanate (69.6g., 0.4m.) and Alfol 6 (40.8g., 0.4m.) (with a strong exotherm to 80°C.), and 0,0'-di-tridecyl dithiophosphoric acid (216g., 0.4m.) to yield 321g. (98.5%) of a light green viscous liquid containing 3.95%P (theory 4.03%).

Timken O.K. load = 40 lbs.

#### EXAMPLE 18

The procedure of Example 16 was repeated using toluene di-isocyanate (69.6g., 0.4m.), 2-ethylhexanol (52.0g., 0.4m.), and 0,0'-di-tridecyl dithiophosphoric acid (216g., 0.4m.) to yield 327g. (98%) of a very light green mobile liquid containing 3.74%P (theory 3.89%).

Timken O.K. load = 50 lbs.

#### EXAMPLE 19

The procedure of Example 16 was repeated using toluene di-isocyanate (69.6g., 0.4m.) 3,5,5-trimethylhexanol (57.6g., 0.4m.), and 0,0'-di-isobutyl dithiophosphoric acid (106.8g., 0.4m.) to yield 211g. (90.5%) of a light green solid containing 5.63%P (theory 5.22%).

Timken O.K. load = 40 lbs.

#### EXAMPLE 20

Isodecanol (79g., 0.5m.) was added to toluene di-isocyanate (87g., 0.5m.) over  $\frac{1}{4}$  hour. The initial temperature was 50°C., exotherming strongly to a maximum 105°C. The reaction mixture was cooled to 80°C. and stirred for a further  $\frac{1}{4}$  hour. 0,0'-di-isobutyl dithiophosphoric acid (134g., 0.5m.) was then added over  $\frac{1}{4}$  hour, keeping the temperature at 75°-80°C., and the mixture stirred for a further  $\frac{1}{4}$  hour, whereafter isodecanol (7.9g., 10%) was added to ensure completion of reaction. There was obtained 201g. (96%) of a light green fairly mobile liquid containing 5.3%P (theory 5.4%).

Timken O.K. load = 40 lbs.

#### EXAMPLE 21

In a manner identical to Example 20, except that a dry nitrogen stream was passed through the reaction mixture to prevent moisture absorption by toluene di-isocyanate, there was prepared from toluene di-isocyanate (435g., 2.5m.), isodecanol (395g., 2.5m.)

and 0,0'-di-isobutyl dithiophosphoric acid (670g., 2.5m.) a clear, light green liquid containing 5.45%P and 12.0%S (theory 5.4% and 11.15% respectively).

#### EXAMPLE 22

This was a repetition of Example 21, identical in every respect, and the product contained 5.3%P and 12.0%S.

Timken O.K. load = 40 lbs.

#### EXAMPLE 23

An 0,0'-di-PIB phenyl dithiophosphoric acid was prepared from  $P_2S_5$  and a polyisobutyl substituted phenol of molecular weight 450. The 0,0'-di-PIB phenyl dithiophosphoric acid (117g., 0.1m.) was added to toluene di-isocyanate (17.4g., 0.1m.) with the temperature at 70°C. and the reaction mixture was stirred for 20 minutes. Isobutanol (7.4g., 0.1m.) was then added and reaction continued for a further  $\frac{1}{2}$  hour to yield a golden brown liquid containing 2.48%P (theory 2.50%).

#### EXAMPLE 24

Phenyl isocyanate (23.8g., 0.2m.) was weighed carefully into a flask and 0,0'-di-isobutyl dithiophosphoric acid (52.6g., 0.2m.) slowly added thereto. The resulting reaction was vigorously exothermic, causing a maximum temperature of 90°C. to be obtained. Stirring was continued for  $\frac{1}{4}$  hour and the final product was a dark green liquid.

#### EXAMPLE 25

Toluene di-isocyanate (17.4g., 0.1m.) was placed in a flask and 0,0'-di-isobutyl dithiophosphoric acid (26.8g., 0.1m.) added thereto. The reaction mixture was stirred at 70°-80°C. for 1½ hours and then tridecanol (20g., 0.1m.) added thereto and stirred for a further hour. The final product was a very viscous, almost colourless liquid containing 5.3%P (theory 5.3%).

#### EXAMPLES 26 TO 31

Further examples were carried out in a similar manner to Example 1, the relevant details of these further examples being set out in Table 1 hereinafter.

The products of various of the foregoing Examples 1 to 31 were tested for suitability as lubricant additives, as also were five prior art additives in accordance with U.S. Pat. No. 3,537,998. The prior art additives were prepared as follows:

Additive 1. [Toluene-2,4-dis-(S-carbamoyl-0,0'-di-2-hexadecyl dithiophosphate)]

Toluene di-isocyanate (17.4g., 0.1m.) was placed in a flask and 0,0'-di-hexadecyl dithiophosphoric acid (127g., 0.2m.) added thereto, the acid being added warm from a beaker due to its waxy nature when cold. The addition of the dithiophosphoric acid produced an exotherm. After completion of the addition the reaction mixture was heated to 70°-80°C. for 2½ hours, to yield a cloudy, quite viscous liquid containing 4.63%P (theory 4.66%). The product solidified after standing overnight.

Additive 2. [Toluene-2,4-di-(S-carbamoyl-0,0'-di-tridecyl dithiophosphate)]

Toluene di-isocyanate (7.81g., 0.066m.) was added dropwise to 0,0'-di-tridecyl dithiophosphoric acid (44.5g., 0.09m.) at 70°-80°C., an exotherm being noticed after each addition. Reaction was continued for

1 1/2 hours at 70°-80°C. to yield a very pale green liquid containing 5.35%P and 10.3%S (theory 5.34% and 11.03% respectively).

Additive 3. [Toluene-2,4-di-(S-carbamoyl-0,0'-di-p-nonylphenyl dithiophosphate)]

0,0'-di-p-nonylphenyl dithiophosphoric acid (54.5g., 0.1m.) was added in small increments to a well-stirred solution of toluene di-isocyanate (8.71g., 0.05m.) in benzene (65ml.). The rate of addition was such that the resulting exotherm did not raise the reaction temperature above 25°C., the temperature being maintained below 25°C. throughout. After completion of the addition the product was vacuum stripped to remove the solvent and the final product was a light green viscous liquid containing 5.10%P and 10.16%S (theory 5.05% and 9.39% respectively).

Additive 4. [Toluene-2,4-di-(S-carbamoyl-0,0'-di-2-ethylhexyl dithiophosphate)]

This was prepared in a similar manner to Additive 3, from 0,0'-di-2-ethylhexyl dithiophosphoric acid (50.0g., 0.133m.) and a solution of toluene di-isocyanate (11.45g., 0.066m.) in benzene (25ml.) The resulting additive was a mobile, green liquid containing 6.72%P and 4.48%S (theory 7.03% and 14.35% respectively).

Additive 5. [Toluene-2,4-di-(S-carbamoyl-0,0'-di-octylphenyl dithiophosphate)]

This additive was also prepared in a similar manner to Additive 3, from 0,0'-di-octylphenyl dithiophosphoric acid (202.4g., 0.4m.) and a solution of toluene di-isocyanate (34.8g., 0.2m.) in benzene (80ml.). The resulting additive was a viscous, light green liquid containing 4.70%P and 10.58%S (theory 5.23% and 10.80% respectively).

In order to evaluate the antiwear (load-carrying) properties of the additives of the present invention the products of a number of the preparations exemplified above were tested by means of the Timken O.K. load test in accordance with the Institute of Petroleum's Test Method IP/240/69. The apparatus employed comprises a roller mounted on a spindle, the roller being rotated against a seated metal block lubricated with the test blend. Also mounted on the spindle is a lever system to one end of which is applied a weight, the weight being increased until the test blend fails as judged by scoring of the seated metal block. The blends tested consisted of sufficient of the test additives to provide a phosphorus content of 0.072% by weight in a base oil which was 150 Solvent Neutral mineral oil having viscosities of about 33 and 5 cSt at 100°F. and 210°F. respectively. The base oil alone had a Timken O.K. load of 12 lbs. and the results obtained with the various test additives are as set out above in each relevant example. Typical results obtained in this test with the widely used zinc 0,0'-di-hydrocarbyl dithiophosphates, at 0.08% by weight phosphorus level, are 33 lbs. (hydrocarbyl = mixed isobutyl and pentyl groups), 35 lbs. (hydrocarbyl = mixed isopropyl and capryl groups) and 12 lbs. (hydrocarbyl = alkyl-phenyl group).

For a qualitative demonstration of antioxidant prop-

erties various blends were tested by means of the Rotary Bomb test carried out at 150°C. and in the presence of water in the manner described in the left-hand column of page 220 of the article entitled "Evaluation of Antioxidants for Automotive Lubricants Using the Rotary Bomb" in the Journal of the Institute of Petroleum Vol. 55, No. 544, July 1969, Pages 219 to 226. The blends tested consisted of a base oil and sufficient of the products of the examples to provide a phosphorus content of 0.072% by weight, the results obtained being as follows:

|                                   | Time to<br>Induction Break |
|-----------------------------------|----------------------------|
| Base Oil only*                    | 45 min.                    |
| Base oil + product of Example 1.  | 122 min.                   |
| Base oil + product of Example 2.  | 78 min.                    |
| Base oil + product of Example 3.  | 402 min.                   |
| Base oil + product of Example 26. | 129 min.                   |
| Base oil + product of Example 27. | 88 min. $\oplus$           |
| Base oil + Additive 4.            | 405 min.                   |
| Base oil + Additive 2.            | 298 min.                   |
| Base oil + Additive 3.            | 82 min. $\oplus$           |
| Base oil + Additive 5.            | 124 min.                   |

\*500 Solvent Neutral mineral oil having viscosities of about 110 and 11 cSt. at 100°F. and 210°F. respectively.

$\oplus$  to 25 p.s.i. loss.

25 Engine tests and tests on a Cam and Tappet machine to simulate in service performance of blends containing the additives of the present invention were also carried out. The engine tests indicated that the additives of the present invention were comparable in efficiency with the widely used zinc 0,0'-di-hydrocarbyl dithiophosphates and good results were obtained on the Cam and Tappet machine.

30 To test Thermal Stability (deposit forming tendencies) blends of base oil (same as in Timken O.K. load tests) containing sufficient of various additives to provide a phosphorus content of 0.5% by weight, were placed in pyrex test tubes (50ml. of test blend in each). The test tubes were then suspended for 1 hour in an oil bath maintained at a temperature of 175° - 180°C. so that about 1 inch of the blend was showing above the surface of the oil bath.

35 Meanwhile, sintered glass crucibles had been cleaned, flushed through with acetone, dried in an oven at 100°C. for about 1/2 hour, cooled in air and weighed.

40 After completion of the 1 hour immersion period, each blend was poured into approximately 200ml. of heptane and the resulting mixture filtered as quickly as possible through a crucible. The crucible contents were then thoroughly rinsed with clean heptane to ensure all oil was removed, then dried in the oven for about 1/2 hour, cooled in air and re-weighed. The results obtained were expressed as the weight of precipitate collected/weight of additive in blend X 100%.

45 In this way were evaluated blends containing one of the aforesaid prior art additives and blends containing the product of Example 25, the results being as follows:

|                                         |         |
|-----------------------------------------|---------|
| Blends containing prior art additive    | 3.92% * |
| Blends containing Product of Example 25 | 0.65% * |

\* mean value of duplicate tests.

TABLE I

| EX.<br>NO. | Isocyanate      | Dithiophosphoric<br>Acid  | Reaction<br>Temp.<br>(°C.) | Product               | Additional<br>Notes               | %P in Product |        | %S in Product |        |
|------------|-----------------|---------------------------|----------------------------|-----------------------|-----------------------------------|---------------|--------|---------------|--------|
|            |                 |                           |                            |                       |                                   | Found         | Theory | Found         | Theory |
| 26         | Ethyl<br>27.6g. | di-p-nonylphenyl<br>206g. | 70-80                      | olive green<br>liquid | Isocyanate added over<br>1/2 hour | 5.14          | 5.12   | 10.3          | 10.58  |

TABLE I—Continued

| EX.<br>NO. | Isocyanate                              | Dithiophosphoric<br>Acid <sup>1</sup>        | Reaction<br>Temp.<br>(°C.) | Product                 | Additional<br>Notes                                                                                                                                                                                                                       | %P in Product |        | %S in Product |        |
|------------|-----------------------------------------|----------------------------------------------|----------------------------|-------------------------|-------------------------------------------------------------------------------------------------------------------------------------------------------------------------------------------------------------------------------------------|---------------|--------|---------------|--------|
|            |                                         |                                              |                            |                         |                                                                                                                                                                                                                                           | Found         | Theory | Found         | Theory |
| 27         | (0.4m.)<br>t-Butyl<br>29.7g.<br>(0.3m.) | (0.4m.)<br>di-tridecyl<br>154.8g.<br>(0.3m.) | 80-85                      | grey/green<br>liquid    | Isocyanate added over<br>½ hour and product<br>reacted at 70°C. for<br>further one hour.                                                                                                                                                  | 5.17          | 5.23   | 10.79         | 10.80  |
| 28         | t-Butyl<br>29.7g.<br>(0.3m.)            | di-p-nonylphenyl<br>154.5g.<br>(0.3m.)       | 70-80                      | yellow<br>liquid        | Isocyanate added over<br>½ hour and product<br>reacted at 70°C. for<br>further one hour.                                                                                                                                                  | 5.09          | 4.82   | 8.89          | 9.95   |
| 29         | t-Octa-<br>decyl<br>118g.<br>(0.4m.)    | di-tridecyl<br>213g.<br>(0.4m.)              | 20-40                      | —                       | Isocyanate added over<br>¾ hour and reaction<br>continued for further<br>1½ hours with temp.<br>gradually returning<br>to 20°C.                                                                                                           | 3.70          | 3.93   | —             | —      |
| 30         | t-Octa-<br>decyl<br>118g.<br>(0.4m.)    | di-isobutyl<br>107g.<br>(0.4m.)              | 20-35                      | —                       | Isocyanate added over<br>¾ hour and reaction<br>continued for further<br>one hour. Small solid<br>particles noticed and<br>filtered off, but<br>further precipitate<br>formed subsequently and<br>whole product eventually<br>solidified. | 5.66          | 5.78   | —             | —      |
| 31         | Allyl<br>8.3<br>(0.1m.)                 | di-isodecyl<br>47g.<br>(0.1m.)               | 20-45                      | mobile<br>yellow liquid | Acid added dropwise to<br>isocyanate at room<br>temperature resulting in<br>exotherm to 45°C<br>Stirred for 2½ hours                                                                                                                      | 6.52          | 6.2    | 13.9          | 12.9   |

We claim:

1. A lubricant composition consisting essentially of lubricating oil having dissolved therein from about 0.1 to 10% by weight of at least one oil-soluble dithiophosphoric acid derivative having the general formula:



wherein  $R^3$  is selected from the group consisting of mono-valent aliphatic groups, mono-valent aromatic groups, di-valent aliphatic groups and di-valent aromatic groups;  $X$  is selected from the group consisting of oxygen atoms and sulphur atoms;  $R^4$  is an alkyl group;  $R^1$  and  $R^2$  are the same or different and are selected from the group consisting of alkyl groups, alkaryl groups, aryl groups, aralkyl groups and alkenyl groups; and  $n$  is 0 when  $R^3$  is a mono-valent group and  $n$  is 1 when  $R^3$  is a divalent group.

2. A composition according to claim 1 wherein  $R^1$  and  $R^2$  are selected from the group consisting of alkyl, alkaryl and aralkyl groups containing from 4 to 18 carbon atoms.

3. A composition according to claim 1 wherein  $R^4$  is an alkyl group containing from 4 to 13 carbon atoms.

4. A composition according to claim 1 wherein  $R^3$  is selected from the group consisting of a mono-valent alkyl group containing from 1 to 18 carbon atoms and a divalent aryl group.

5. A composition according to claim 4 wherein  $R^3$  is a divalent aryl group bearing at least one alkyl substituent and containing from 6 to 24 carbon atoms.

30 6. A composition according to claim 1 containing from 0.5 to 5% by weight of the dithiophosphoric acid derivatives.

35 7. A composition according to claim 1 containing in addition to the dithiophosphoric acid derivatives, from about 0.1 to 5% of a compound selected from the group consisting of mono-octyl phenyl- $\alpha$ -naphthylamines, mono-octyl phenyl- $\beta$ -naphthylamines, mono-nonyl phenyl- $\alpha$ -naphthylamines and mono-nonyl phenyl- $\beta$ -naphthylamines.

40 8. An oil concentrate or additive package comprising from 10% to 70% by weight of a lubricating oil having dissolved therein from 90% to 30% by weight of at least one dithiophosphoric acid derivative having the formula:



45 55 wherein  $R^3$  is selected from the group consisting of mono-valent aliphatic groups, mono-valent aromatic groups, di-valent aliphatic groups and di-valent aromatic groups;  $X$  is selected from the group consisting of oxygen atoms and sulphur atoms;  $R^4$  is an alkyl group;  $R^1$  and  $R^2$  are the same or different and are selected from the group consisting of alkyl groups, alkaryl groups, aryl groups, aralkyl groups and alkenyl groups; and  $n$  is 0 when  $R^3$  is a mono-valent group and  $n$  is 1 when  $R^3$  is a di-valent group.

60 \* \* \* \* \*